

## UNITED STATES PATENT OFFICE

2,397,193

WOOD BLEACH AND PROCESS OF MAKING  
SAME

Gustavus Harry Miller, Portland, Oreg.

No Drawing. Application May 15, 1942,  
Serial No. 443,170

3 Claims. (Cl. 252—99)

This invention relates to bleaching wood and more particularly to bleaching the surfaces of plywood and hardwood veneers used in the wood-working and furniture industries, the principal object being to provide a bleach that will lighten dark wood surfaces to a uniform color, at ordinary temperatures without distorting the wood surface or unduly raising the grain, or otherwise rendering the surface unfit for application of finishing coatings immediately following the bleaching operation.

Another object of this invention is to provide an economical, quick acting and quick-drying odorless bleach which, when sprayed, will penetrate the surface of the wood sufficiently to provide a permanently and uniformly bleached surface, in one operation, which does not require cleaning or the application of alcohol as a neutralizer before applying the finishing materials. Such simple methods of application as spraying, brushing, or dipping are used without regard to time and temperature regulation. Soaking or immersing the material for long periods of time as in former bleaching processes is definitely unnecessary and furthermore is undesirable since deep penetration of the liquid into the wood tends to raise the grain thereof.

A further object of this invention is to provide a simple prepared bleaching solution which comprises adding one part by volume hydrogen peroxide solution to an equal portion by volume of an alkali solution and, this combination as an active oxidizing agent will remain relatively stable at normal temperatures for four hours.

In prior art, wooden articles were bleached by the oxidizing action of hydrogen peroxide in a closed system usually at elevated temperatures, together with added amounts of sodium silicate, pyrophosphate, or potassium permanganate, and often in the presence of ammonia. Unevenness of color resulted in the harder portions of the grain and the softer wood fiber, and over-absorption of the bleach solution invariably required after-drying of the wood at additional expense, with a tendency to checking, before finishes could be applied. Wood surfaces were also bleached by the use of a solution containing three parts hydrogen peroxide (30% by weight), to one part by volume of an alkali solution composed of sodium silicate and lime. The early methods were not able to provide a definite pH control and therefore the surface of the wood was either too alkaline or too acid; and, for this reason, alcohol was often used as a neutralizer. Furthermore, due to the sodium tetrasilicate con-

tained in the alkali mixture, a crystallized formation resulted on drying which would not respond satisfactorily to the finishing material.

Another well known process is to use three parts by volume of hydrogen peroxide to one part by volume of ammonium hydroxide.

When ammonia is used as the alkaline solution and hydrogen peroxide as the acid solution, the obnoxious ammonia fumes must be guarded against with proper equipment (masks) to protect the operator from the intolerable irritating fumes.

Now, in accordance with the present invention and as hereinafter described and set forth in the examples of this invention, the bleaching solution composed of a mixture of one part by volume of aqueous hydrogen peroxide (30% by weight), and in equal portion by volume of an alkali solution, an active oxygen producing agent is provided to realize a uniformly bleached surface, without external aids, ready for finishing material, which is relatively stable from four to five hours at normal temperatures (70-75° F.). This practically odorless solution can be applied to the wood surface by either brush, spray, or dip in the usual manner, and although the surface is generally wet sufficiently to obtain a penetration of about one-twentieth inch, it will dry at room temperature in about an hour. Preferred results are obtained at 75 to 85° F., without the aid of ammonia vapor. An additional application is an improvement when very hard or badly stained and difficult types of wood are encountered.

The desired results are obtained within narrow limits as set forth in the following examples:

## Example I

|                                                       | Ounces |
|-------------------------------------------------------|--------|
| Borax (commercial-granulated), weight                 | ½      |
| Caustic soda (NaOH), weight                           | 1      |
| Water, volume                                         | 6      |
| Waterglass (sodium tetrasilicate, 42° Bé.),<br>volume | %      |
| Water, volume                                         | 3½     |

The borax is added to an 800 cc. beaker with the caustic soda on top; six ounces of water are slowly added with constant stirring; when dissolved, add the sodium tetrasilicate and follow with the balance of the water. Let stand over night to cool and clear up. Decant or syphon off the crystal-clear liquid.

The foregoing aqueous alkaline solution with a pH of 10.7 is added in equal volume to an aqueous hydrogen peroxide solution (30% by weight) with a pH of 2.5 immediately prior to application to the wood surface. The combined solutions have an initial pH of 9.7 and will retain their bleaching properties for four hours at normal temperatures; applied as a bleach to the wood, the surface, when dry, will be free from residue and require no neutralizing before applying the finishing materials.

#### Example II

An aqueous solution containing:

|                                   | Pounds |
|-----------------------------------|--------|
| Borax (sodium tetraborate)        | 1      |
| Caustic soda (sodium hydroxide)   | 2      |
| Sodium tetrasilicate              | 1      |
| Water                             | 20     |
| Hydrogen peroxide (30% by weight) | 24     |

is prepared in a ten gallon mixing tank provided with an agitator; such equipment should be made to withstand the corrosive action of an aqueous caustic solution and the agitator geared to a speed sufficient to keep the materials from settling to the bottom until dissolved.

Add the water to the mixing tank and start the agitator, then slowly add the borax, sodium hydroxide, and sodium tetrasilicate; when dissolved, draw off the aqueous alkaline solution into a settling tank to cool and clear up before filling into stock containers which are usually glass bottles closed with a rubber stopper.

Twenty-four pounds of the above alkaline solution is added to twenty-four pounds of an aqueous hydrogen peroxide solution (30% by weight) immediately prior to application to the wood surface as a colorless, odorless wood bleach to provide a bleached surface free from residue that does not require neutralizing before applying such finishing materials as woodstains, fillers, clear primers, varnish, or lacquer.

#### Example III

An aqueous solution containing:

|                                 | Pounds |
|---------------------------------|--------|
| Borax (sodium tetraborate)      | 1      |
| Caustic soda (sodium hydroxide) | 2      |
| Sodium tetrasilicate            | 1      |
| Water                           | 21     |

is prepared in a mixing tank provided with a spigot two inches from the bottom and equipped with an agitator, the speed of which shall be sufficient to keep the materials from settling to the bottom while mixing. Such equipment should be made of material that will withstand the corrosive action of an aqueous caustic solution.

The water is added to the tank and the borax, sodium hydroxide, and sodium tetrasilicate slowly added with constant agitation; when dissolved, the solution is allowed to cool and clear up before filling into stock containers which are often rubber or glass lined or glass bottles with rubber stoppers.

The above composition is added in equal proportion by weight to an aqueous hydrogen peroxide solution (30% by weight) to provide a colorless, odorless wood bleach; which, applied to the wood surface by either spray, brush, or dip, will provide a bleached surface free from residue that requires no neutralizing before applying finishing materials.

#### Example IV

An aqueous solution containing:

|                                                                   |         |        |
|-------------------------------------------------------------------|---------|--------|
| Borax (sodium tetraborate)                                        | pounds  | 12     |
| Na <sub>2</sub> B <sub>4</sub> O <sub>7</sub> ·10H <sub>2</sub> O | do      | 24     |
| Caustic soda (sodium hydroxide)                                   | gallons | 18     |
| NaOH                                                              | do      | 1 1/2  |
| Water                                                             | do      | 10 1/2 |
| Waterglass (sodium tetrasilicate)                                 |         |        |
| Na <sub>2</sub> Si <sub>4</sub> O <sub>9</sub>                    |         |        |
| Water                                                             |         |        |

is made in a mixing tank which may be a synthetic rubber lined wood, iron, or steel barrel provided with a spigot or valve about two inches from the bottom so that the clear liquid can be drawn off without disturbing the residue left on the bottom. A wooden paddle may be used as a stirrer.

15 The borax is added to the mixing tank and the sodium hydroxide is put on top. Eighteen gallons of water are slowly added with constant stirring; when dissolved, add the sodium tetrasilicate and follow with the balance of the water. Let stand over night to cool and clear up. It is now ready to draw off into suitable containers.

The above described solution with a pH of 10.9 is added to an equal volume of an aqueous hydrogen peroxide solution with a pH of 2.5; at the time the two solutions are combined as a bleach, they will have a pH of 9.7; one hour later, a pH of 9.8; two hours later, a pH of 9.9 which remains quite constant for three hours at a room temperature of 68-72° F.; usually after twenty-four hours, the bubbling subsides and the final pH 30 value is 10.9; applied to either hard or soft wood surfaces, the combined solutions apparently undergo an accelerated reaction whereby the oxidation or bleaching is accomplished in less than an hour at 75-80° F. within a pH range from 9.7 at the time of application to a pH of 10.9 at the time of exhaustion. The definite action in the bleaching process is achieved by reason of the materials used in the proportions as prescribed 35 in the examples and set forth in the claims; the sodium ion activates the oxidation at the surface when in solution with hydrogen peroxide and the sodium ion is greatly enhanced when a hydrogen ion is also in solution. Borax and sodium tetrasilicate in the proportions indicated 40 50 in the examples are both used as mild activators of hydrogen peroxide and as buffering agents to retard the action of the sodium ion on the cellulose and poly-saccharose compounds in wood. The reaction, when completed, leaves no ash or residue on the wood surface which has the final 55 appearance of having been cleaned and bleached to a uniform color.

#### Example V

60 An aqueous solution containing:

|                                   |         |    |
|-----------------------------------|---------|----|
| Borax (sodium tetraborate)        | pounds  | 21 |
| Caustic soda (sodium hydroxide)   | do      | 43 |
| Waterglass (sodium tetrasilicate) | gallons | 2  |
| Water                             | do      | 51 |

is prepared by adding the borax and caustic soda to a suitable mixing tank; fifty-one gallons of water are slowly added with constant stirring until the materials are completely dissolved; the sodium tetrasilicate is dispersed in the solution, and the agitator is stopped to allow the liquid to cool and clear up.

The mixing tank may be made of iron or steel and lined with a non-corrosive material such as 75 Pyrex glass or synthetic rubber, equipped with a

suitable agitator of a corrosion-proof metal with provision made for drawing off the liquid so that the impurities as sediment which collects on the bottom of the tank are not disturbed. The residue is removed and the tank is washed after each operation.

The above described solution with a pH of 10.5-11 is added to an equal volume of hydrogen peroxide solution with a pH of 4-5; within five minutes from the time of combining the two solutions, a fairly constant pH of 9.5-10 is reached and shows little change for about four hours. After a period of twenty-four hours, the oxygen has been practically expelled and the solution has a pH of 10.5-11.

By reason of the buffer action brought about by the given proportions of waterglass and borax, the action of the sodium ion on the wood fibre is such as to bring about the optimum conditions for an oxidizing action on the wood surface. The definite action in the bleaching process is achieved by the admixture of the materials in the proportions as prescribed in the examples and set forth in the claims.

Although the present invention has been described in the foregoing examples with specific details, it is not intended that such details shall be regarded as limitations upon the scope of the invention, except insofar as is included in the accompanying claims.

What I claim is:

1. A method of bleaching smooth wood surfaces which have been otherwise finally conditioned for receiving finishing coatings without adversely affecting such surfaces which comprises applying a thin film of a bleach solution consisting of about one volume of an alkali component consisting substantially of one part by weight borax, two parts by weight caustic soda, one part by weight 42° Bé. waterglass, twenty parts by weight water, and a second component consisting of a substantially equal volume of hydrogen peroxide (30% by weight), said two components having been mixed together substantially immediately before the ap-

plication thereof to said wood surface, permitting said wood surface to dry at room temperature after the application of said film thereto whereby said wood surface is left smooth, free from residue, and in condition for immediately receiving finishing coatings.

2. A method of bleaching a smooth wood surface which will leave the surface clean, free of rough crystalline residue, substantially neutral and otherwise unaltered as concerns the application of finishing coatings onto the bleached surface, which method comprises spraying onto the wood surface a thin film of a bleach solution consisting substantially of a freshly mixed mixture of equal volumes of hydrogen peroxide (30% by weight) and an alkaline solution consisting of one part by weight borax, two parts by weight caustic soda, one part by weight 42° Bé. waterglass, and twenty parts by weight water, and allowing said wood surface to dry thereafter at room temperature to minimize penetration of the solution into the wood whereby the grain of the wood is not raised and the surface of the wood left clean and smooth.
- 10 3. A bleaching solution for bleaching smooth wood surfaces which have been otherwise finally conditioned for receiving finishing coatings which solution consists of a mixture of two substantially equal volumes of previously prepared components, one of said components consisting substantially of one part by weight borax, two parts by weight caustic soda, one part by weight 42° Bé. waterglass, 20 parts by weight water, the second component consisting of hydrogen peroxide (30% by weight), said solution being adapted for spray application onto said wood surface immediately after the mixing of said two components and being characterized by the fact that upon drying of said wood surface at room temperature following such application, said wood surface is left smooth, free from residue and in condition for immediately receiving finishing coatings.
- 15 20 25 30 35 40

G. HARRY MILLER.